

1,186,055.

F. S. WHITE.  
METHOD OF MAKING STAMP SHOES.  
APPLICATION FILED MAR. 19, 1915.

Patented June 6, 1916.

2 SHEETS—SHEET 1.



FIG. 1.



FIG. 2.



FIG. 3.

FIG. 4.



FIG. 5.



WITNESSES:

*Bob A. Mitchell*  
E. E. Hall

INVENTOR

*Francis S. White*  
BY *Frank J. Busser*  
ATTORNEY.

1,186,055.

F. S. WHITE.  
METHOD OF MAKING STAMP SHOES.  
APPLICATION FILED MAR. 19, 1915.

Patented June 6, 1916.  
2 SHEETS—SHEET 2.



WITNESSES:

P. H. Stetich  
E. E. Hall

INVENTOR

Francis S. White  
by  
Frank J. Quisen  
ATTORNEY.

# UNITED STATES PATENT OFFICE.

FRANCIS S. WHITE, OF PHILADELPHIA, PENNSYLVANIA.

## METHOD OF MAKING STAMP-SHOES.

1,186,055.

Specification of Letters Patent.

Patented June 6, 1916.

Application filed March 19, 1915. Serial No. 15,413.

To all whom it may concern:

Be it known that I, FRANCIS S. WHITE, a citizen of the United States, residing at Philadelphia, county of Philadelphia, and

5 State of Pennsylvania, have invented a new and useful Improvement in Methods of Making Stamp-Shoes, of which the following is a full, clear, and exact description, reference being had to the accompanying 10 drawings, which form a part of this specification.

The object of my invention is the economical production of stamp shoes of fine quality.

15 My process may be carried out in different ways, but I prefer to carry it out in the manner and with the apparatus illustrated in the drawings, in which—

Figure 1 is a side view, and Fig. 2 a cross-section of an ordinary ingot. Fig. 3 is a side view showing the shape to which a section of the ingot is forged. Fig. 4 is a side view of the finished product. Fig. 5 is a vertical section of the die employed in the 25 final operation. Fig. 6 is a vertical longitudinal section, and Fig. 7 a cross section (on line 7—7 of Fig. 6), of the forging die, the ingot section being shown in its original condition; Fig. 8 being a view similar to 30 Fig. 7, but showing the article shaped in conformity with Fig. 3.

Initially, I take an ingot *a* and cut the same into sections of equal mass on the lines *x*, *x*. An ingot section *b* is then placed between die members *c* and *d* (see Figs. 6 and 35 7). These die members are provided at one end with inwardly extending flanges *e* forming an abutment to prevent flow of the metal in one direction. The die members 40 from their flanged or closed ends have parallel walls, while toward their opposite ends the walls converge as shown in Fig. 6. The walls of the die are cut away at *f* to permit of the entrance of a tool *g* whereby the piece 45 may be turned.

In operation, the upper die member is

alternately lifted and depressed, the piece being turned after each action, thereby reducing its cross section and causing the metal thereof to flow toward the narrow 50 mouth of the die. The piece is turned from time to time. At the conclusion of the forging operation, the piece is shaped to conform to the forging die, as shown at *h*, Fig. 3. It is then placed upon the lower die 55 member *h* of Fig. 5, which, in conjunction with upper die member *i* and plunger *j* shapes the piece to its ultimate form, as shown at *m*, Fig. 4. This operation, which is an upsetting one, increases the diameter, 60 and shortens the length, of both the body and the neck of the piece, besides flattening the shoulder between the body and neck.

Having now fully described my invention, what I claim and desire to protect by Letters Patent is:

1. The process of making stamp shoes, which consists in casting the piece, applying a forging pressure thereto in a radial direction while causing the metal at one end to 70 flow longitudinally to form a neck of smaller diameter, and then compressing the same longitudinally and squaring the shoulder between head and neck.

2. The process of making stamp shoes, 75 which consists in casting the piece, applying a forging pressure in a radial direction thereto while limiting the longitudinal flow of the metal in one direction and causing it to flow longitudinally in the other direction 80 to form a contracted neck joined to the body by a sloping wall, and then compressing the same longitudinally and squaring the shoulder between head and neck.

In testimony of which invention, I have 85 hereunto set my hand, at Philadelphia, on this 12th day of March, 1915.

FRANCIS S. WHITE.

Witnesses:

J. ENTWISLE,  
ARTHUR KRONEMANN.

Copies of this patent may be obtained for five cents each, by addressing the "Commissioner of Patents, Washington, D. C."